

## UNITED STATES PATENT OFFICE

LAWRENCE BRADSHAW, OF BAINBRIDGE, NEW YORK, ASSIGNOR TO THE CASEIN MANUFACTURING COMPANY OF AMERICA, INC., OF NEW YORK, N. Y., A CORPORATION OF DELAWARE

## ADHESIVE AND PROCESS OF MAKING SAME

No Drawing.

Application filed January 2, 1930. Serial No. 418,164.

This invention relates to improving the quality of cheap adhesives or glues made from peanut meal, slaked lime and alkali metal salts with or without additional cellulose substances such as wood meal, hull meal or other filling materials such as ground leather scrap.

I have previously described a glue suitable for gluing up plywood and the like, prepared from peanut meal, slaked lime and sodium salts which latter have the property of reacting with lime to produce insoluble salts of calcium and liberate caustic soda. This glue can conveniently be made up in a dry state at the factory and subsequently mixed with water when required for use. The peanut meal employed is usually the pulverized press-cake of commerce, commonly sold as a feeding stuff, containing about 43% protein, and 6 to 8% residual oil. For use in glues this meal is usually re-ground so that substantially all of it will pass through a 120 mesh screen, or even finer. One part of the glue base thus prepared can be mixed with about 2 1/8 to 2 1/4 parts of water to make an adhesive of good working qualities for applying to plywood or veneers, the usual practice being to stir the mixture for fifteen to twenty minutes in order to obtain a fluid product of suitable consistency for applying to wood by the machines employed in the art for this purpose.

The object of the present invention is to more fully utilize the insoluble organic ingredients of the glue by causing them to plump or swell up so that a greater portion of water can be used and the volume of the glue increased without undue thinning, the consistency of the glue being maintained; and the glue can be distributed over a larger surface in the subsequent spreading operation. It is based upon the discovery that the addition of caustic soda to the fluid glue after the process of solution of the proteins by the alkali salts of the glue-base is substantially complete, produces a rapid thickening of the glue, which can then be diluted with water to restore it to the desired consistency, resulting in a great increase in the bulk or volume of fluid glue which can be made from a unit

weight of the dry glue base. This thickening is much greater than would be produced by equivalent amounts of soluble sodium salts to the dissolved glue, and I believe that it arises from the swelling action of the free caustic soda on the cellulose and starchy constituents of the glue.

While the peanut meal itself contains a substantial amount of fibre, other cellulose materials such as wood flour, bran, oat hulls, ground corn cobs, ground sugar cane are sometimes added to such meals to act as fillers in the glues, the use of such fillers having proved advantageous in some cases, for instance in the gluing together of soft woods. Such fillers, however, might be a source of weakness rather than of strength where they are insufficiently plumped, and I have found that a comparatively small amount of free caustic soda is a much more effective plumping agent than a larger amount of sodium salts in presence of lime. The sodium salts commonly employed in making up a glue base are the phosphate, carbonate, sulfite and fluoride; the corresponding salts of potassium may likewise be employed.

The following examples will serve to illustrate the method of carrying out the invention, which however is not restricted to these examples.

*Example 1.*—84 parts of peanut meal, 12 parts of hydrated lime and 4 parts of sodium fluoride are mixed together to form a dry glue base. 100 parts of this glue base are then mixed with 350 parts of water at about 70° F. and well stirred for 15 to 20 minutes. Then 7 parts of caustic soda dissolved in 14 parts of water are added and the stirring continued for a short time, say 1 to 5 minutes. This liquid glue will accordingly be seen to contain, with 100 parts of the dry glue base, 364 parts of water, together with 7 parts of NaOH. The amount of water is a little over 3.4 times the total amount of all the other constituents. The glue is then ready to be applied to veneers for the making of plywood. This glue spreads well on the usual machines employed in the art for applying liquid glue.

In this example it will be noted that after 100

mixing the dry glue base with water, in the proportions stated, the glue is very thin, and those familiar with the art would consider the glue at this stage to be too thin for use in 5 gluing up plywood. Within a very short time after adding the caustic soda, however, it will be observed that the glue has thickened to a suitable consistency for this purpose.

10 *Example 2.*—84 parts of peanut meal, 10 parts of hydrated lime, 3 parts of sodium fluoride and 3 parts of tri-sodium phosphate are mixed together dry to form a dry glue base. Subsequently when it is desired to use 15 the glue, the base is mixed with about 3.7 times its own weight of water and stirred for 15 minutes. This produces a thin, liquid glue. 5 parts of caustic soda in the form of a 40% solution are then added and the stirring 20 continued for about 2 minutes, when it will be found that the glue has thickened greatly and acquired a good body or consistency suitable for spreading. This liquid contains, per 100 parts of dry glue base, 377 25 parts of water, together with 5 parts of NaOH. The water is almost 3.6 times the total amount of all the other constituents.

16 *Example 3.*—76 parts of peanut meal, 10 parts of wood flour, 10 parts of hydrated lime, 3 parts of sodium fluoride and 1 part of sodium carbonate are mixed together to form a dry glue base. Subsequently 1 part of this glue base is mixed with about 3.8 parts of water and stirred for about 15 minutes, which 35 produces a very thin-flowing liquid glue. 6 parts of dry caustic soda are sprinkled into the liquid and the stirring continued for 3 to 5 minutes, when the caustic soda passes into solution and the glue thickens to a good, 40 workable consistency. This liquid glue contains, with 100 parts of the dry glue base and 6 parts of caustic soda, 380 parts of water. The water is over 3.5 times the total amount of the other constituents.

45 I call attention to the fact that the caustic soda is added after the initial mixing of the glue powder with the water, preferably not less than 10 minutes after the mixing operation is begun, by which time the protein 50 content of the glue is believed to be substantially all dissolved. The agitation of the glue base with water according to current practice usually requires about 20 minutes.

and I may add the caustic soda preferably after about 15 minutes and continue stirring to the end of the period. The proportion of the caustic soda may vary more or less, say from 3% up to 8% of the weight of the dry 70 glue-base.

I claim:

1. A process of preparing fluid peanut glue which comprises mixing with about 3 $\frac{3}{4}$  parts of water, one part of a peanut glue base comprising a major part of peanut meal, hydrated lime equal to a minor fraction of the peanut meal and a still smaller amount of alkali metal salt capable of reacting with the lime to form insoluble compounds of calcium, and thereafter adding caustic soda 80 to effect a thickening.

2. In the making of fluid peanut glue, the steps of first mixing up with water, a peanut glue base containing comminuted peanut meats from which the bulk of the peanut oil has been removed, sodium salts of acids which form insoluble compounds with lime, and lime, and thereafter, but before use of the glue, adding caustic soda, 85 whereby a substantial thickening of the fluid glue is effected, the total amount of water added being at least 3.5 times the weight 90 of the dry glue base.

3. A process of preparing fluid peanut glue which comprises mixing with not below 3.5 parts of water, 1 part of a peanut glue base, comprising a major part of peanut meal, slaked lime equal to a minor fraction of the peanut meal and a still smaller amount of alkali metal salts capable of reacting with the slaked lime in the presence of water, and thereafter adding caustic alkali to the 100 very thin liquid glue to effect a thickening 105 thereof.

4. A process of making liquid glue of sufficient body for use in making plywood from veneers, which comprises adding a glue base to water, the glue base containing peanut meal as its major constituent together with slaked lime, alkaline sodium salts and sodium fluoride, and after some mixing, adding caustic soda, the caustic soda being in amount equal to about 3 to 8% of the amount of peanut meal, and the amount of water being about 3.5 to 3.8 times the amount of the dry glue base.

LAWRENCE BRADSHAW.